

# United States Patent [19]

Watson et al.

[11]

4,049,426

[45]

Sept. 20, 1977

[54] COPPER-BASE ALLOYS CONTAINING CHROMIUM, NIOBium AND ZIRCONIUM

[75] Inventors: W. Gary Watson, Cheshire; John F. Breedis, Trumbull, both of Conn.

[73] Assignee: Olin Corporation, New Haven, Conn.

[21] Appl. No.: 728,977

[22] Filed: Oct. 4, 1976

[51] Int. Cl.<sup>2</sup> ..... C22F 1/08

[52] U.S. Cl. ..... 75/153; 148/12.7 C;  
148/32.5; 148/160

[58] Field of Search ..... 75/153; 148/12.7 C,  
148/32.5, 160

[56]

## References Cited

### U.S. PATENT DOCUMENTS

|           |         |                      |            |
|-----------|---------|----------------------|------------|
| 3,143,442 | 8/1964  | Watts .....          | 148/160    |
| 3,357,824 | 12/1967 | Saarvita .....       | 148/160    |
| 3,881,965 | 5/1975  | Matsuda et al. ..... | 148/12.7 C |
| 3,969,156 | 7/1976  | Wallbaum .....       | 148/12.7 C |

Primary Examiner—W. Stallard

Attorney, Agent, or Firm—Robert A. Dawson; Robert H. Bachman

[57]

## ABSTRACT

Copper base alloys containing chromium, zirconium and niobium are disclosed as well as a process of heat treating and mechanically working said alloys. The combination of alloying elements, hot and cold working, annealing and aging steps increases both the strength and electrical conductivity properties of the alloy without excessive cold working.

20 Claims, No Drawings

## COPPER-BASE ALLOYS CONTAINING CHROMIUM, NIOBIUM AND ZIRCONIUM

### BACKGROUND OF THE INVENTION

Commercially useful copper base alloys should possess a combination of high strength and high electrical conductivity for most applications. Unfortunately, the methods and elements previously utilized to provide an increase in one of these properties do so at the detriment of the other property. For example, elements such as zirconium and chromium have been used as additions to copper base alloys to provide this desirable combination of high strength and high electrical conductivity. The precipitation of chromium in copper is known to give large increases in strength and electrical conductivity over the values for the solid solution of copper and chromium. The precipitation hardened alloys containing chromium in copper have lower electrical conductivity but higher strength than pure copper. Precipitation of zirconium in copper is known to give large increases in electrical conductivity but only small increases in strength properties over the values for the solid solution of zirconium in copper. Zirconium also significantly raises the recrystallization temperature of copper. These alloys have lower electrical conductivity properties than pure copper but a much better resistance to softening at high temperatures than pure copper.

Vanadium has recently been utilized to provide the combination of high strength and high electrical conductivity. For example, copending application Ser. No. 652,997 filed Jan. 28, 1976 discusses the effects of adding vanadium to copper base alloys containing chromium and zirconium. Russian Pat. No. 185,068 also discloses copper base alloys that contain chromium, zirconium and vanadium. This patent does not teach any processing steps for this alloy combination.

The present invention is an attempt to overcome the shortcomings of the alloy system described above by combining niobium with copper base alloys containing chromium and zirconium in order to increase the electrical conductivity of the alloys without detrimentally affecting the strength or hardness properties of said alloys.

Accordingly, it is a principal object of the present invention to provide an alloy system which is capable of improving the electrical conductivity without lowering the strength properties of said alloy system.

It is an additional object of the present invention to provide a process for treating the alloy system as aforesaid to develop the electrical conductivity and strength properties thereof.

Further objects and advantages of the present invention will become more apparent from a consideration of the following specification.

### SUMMARY OF THE INVENTION

In accordance with the present invention it has been found that the foregoing objects and advantages may be readily achieved by providing a copper base alloy system containing 0.05 to 1.25% by weight chromium, 0.05 to 1.0% by weight zirconium, 0.05 to 1.5% by weight niobium, balance essentially copper.

This alloy system may be processed according to the following steps:

- a. casting a copper base alloy containing 0.05-1.25% by weight chromium, 0.05-1.0% by weight zirco-

- nium, 0.05-1.5% by weight niobium, balance essentially copper;
- b<sub>1</sub>. hot working the alloy at a starting temperature of 850°-950° C; or
  - b<sub>2</sub>. hot working the alloy at a starting temperature of 950°-1000° C to effect the maximum solid solution of all alloying elements;
  - c. if step (b<sub>1</sub>) has been utilized, solution annealing the worked alloy at a solutionizing temperature of 950°-1000° C, preferably 975°-1000° C, for a period of time sufficient to insure the maximum solid solution of the alloying elements;
  - d. rapidly cooling the alloy to maintain said maximum solid solution of all alloying elements;
  - e. cold working the alloy to a total reduction of at least 60 percent and preferably to at least 75 percent;
  - f. aging said alloy at 400°-500° C for one to 24 hours and preferably 430°-470° C for 2 to 10 hours; and
  - g. optionally cold working said alloy to the final desired temper.

### DETAILED DESCRIPTION

The present invention provides its combination of strength and electrical conductivity properties through a combination of the novel alloy system and the steps of casting this alloy system, hot working the alloy at 850°-950° C or hot working the alloy in such a manner so as to effect the maximum solid solution of all alloying elements, solution annealing the hot worked alloy, if hot worked at 850°-950° C, rapidly cooling the alloy so as to maintain said maximum solid solution, cold working the alloy and aging the alloy.

The hot working step of the processing utilized in the present invention may by itself be used to provide the effect of solution annealing. This is generally accomplished by performing the hot working at a temperature which is high enough to place all of the alloying elements into maximum solid solution. This temperature should be at least 950° C with a preferred temperature range of 975°-1000° C to insure said maximum solid solution.

The alloys utilized in said process are generally cast at a temperature which ranges between 25° C above the melting point of the alloy up to approximately 1300° C. This casting may be performed by any known and convenient method.

The hot working reduction requirement is generally what is most convenient for further working. The process utilized in the present invention has no particular dimensional requirements other than that the hot working be accomplished according to good mill practice. If the hot working step is also utilized to provide the solution annealing of the alloy, the main consideration is that the hot working be performed to effect the maximum solid solution of all the alloying elements. This permits the later precipitation during aging of the most desirable high volume fraction of fine uniform dispersions of intermediate solid phases consisting of chromium, zirconium and niobium, the phases existing in the alloy matrix either as dependent or intermixed phases. The solution annealing step of the process utilized in the present invention, whether performed as part of the hot working step or as a separate step after hot working, also provides for the maximum solid solution of all the alloying elements. This solution annealing is accomplished at a temperature between 950° and 1000° C. It is preferred that the solution annealing be accomplished at

a temperature between 975° and 1000° C. It should be noted that this solution annealing step can take place at any point in the instant process after the initial hot working step, provided that rapid cooling, cold working and aging steps with optional cold working after aging are performed after the solution annealing step.

The alloy, after being either hot worked alone or hot worked in combination with a separate solution annealing step, is then rapidly cooled so as to maintain the maximum solid solution of all alloying elements. Cooling to 350° C or less is necessary to maintain said maximum solid solution. This cooling may be accomplished according to procedures well known in this art, using either air or liquid as the cooling medium.

The next step in the process utilized in the present invention is cold working of the alloy. This cold working step is utilized to provide an increase in strength to the alloy as well as being used to meet dimensional requirements. The alloy is generally cold worked to an initial reduction of at least 60 percent and preferably at least 75 percent. This relatively high cold reduction serves to impart more strain hardening to the alloy prior to aging as well as impart improvement in the electrical conductivity of the aged alloy. The improvement in electrical conductivity after aging of the alloy is pre-

10

20

25

40

45

50

55

60

65

56  
61  
66  
71  
76  
81  
86  
91  
96  
101  
106  
111  
116  
121  
126  
131  
136  
141  
146  
151  
156  
161  
166  
171  
176  
181  
186  
191  
196  
201  
206  
211  
216  
221  
226  
231  
236  
241  
246  
251  
256  
261  
266  
271  
276  
281  
286  
291  
296  
301  
306  
311  
316  
321  
326  
331  
336  
341  
346  
351  
356  
361  
366  
371  
376  
381  
386  
391  
396  
401  
406  
411  
416  
421  
426  
431  
436  
441  
446  
451  
456  
461  
466  
471  
476  
481  
486  
491  
496  
501  
506  
511  
516  
521  
526  
531  
536  
541  
546  
551  
556  
561  
566  
571  
576  
581  
586  
591  
596  
601  
606  
611  
616  
621  
626  
631  
636  
641  
646  
651  
656  
661  
666  
671  
676  
681  
686  
691  
696  
701  
706  
711  
716  
721  
726  
731  
736  
741  
746  
751  
756  
761  
766  
771  
776  
781  
786  
791  
796  
801  
806  
811  
816  
821  
826  
831  
836  
841  
846  
851  
856  
861  
866  
871  
876  
881  
886  
891  
896  
901  
906  
911  
916  
921  
926  
931  
936  
941  
946  
951  
956  
961  
966  
971  
976  
981  
986  
991  
996  
1001  
1006  
1011  
1016  
1021  
1026  
1031  
1036  
1041  
1046  
1051  
1056  
1061  
1066  
1071  
1076  
1081  
1086  
1091  
1096  
1101  
1106  
1111  
1116  
1121  
1126  
1131  
1136  
1141  
1146  
1151  
1156  
1161  
1166  
1171  
1176  
1181  
1186  
1191  
1196  
1201  
1206  
1211  
1216  
1221  
1226  
1231  
1236  
1241  
1246  
1251  
1256  
1261  
1266  
1271  
1276  
1281  
1286  
1291  
1296  
1301  
1306  
1311  
1316  
1321  
1326  
1331  
1336  
1341  
1346  
1351  
1356  
1361  
1366  
1371  
1376  
1381  
1386  
1391  
1396  
1401  
1406  
1411  
1416  
1421  
1426  
1431  
1436  
1441  
1446  
1451  
1456  
1461  
1466  
1471  
1476  
1481  
1486  
1491  
1496  
1501  
1506  
1511  
1516  
1521  
1526  
1531  
1536  
1541  
1546  
1551  
1556  
1561  
1566  
1571  
1576  
1581  
1586  
1591  
1596  
1601  
1606  
1611  
1616  
1621  
1626  
1631  
1636  
1641  
1646  
1651  
1656  
1661  
1666  
1671  
1676  
1681  
1686  
1691  
1696  
1701  
1706  
1711  
1716  
1721  
1726  
1731  
1736  
1741  
1746  
1751  
1756  
1761  
1766  
1771  
1776  
1781  
1786  
1791  
1796  
1801  
1806  
1811  
1816  
1821  
1826  
1831  
1836  
1841  
1846  
1851  
1856  
1861  
1866  
1871  
1876  
1881  
1886  
1891  
1896  
1901  
1906  
1911  
1916  
1921  
1926  
1931  
1936  
1941  
1946  
1951  
1956  
1961  
1966  
1971  
1976  
1981  
1986  
1991  
1996  
2001  
2006  
2011  
2016  
2021  
2026  
2031  
2036  
2041  
2046  
2051  
2056  
2061  
2066  
2071  
2076  
2081  
2086  
2091  
2096  
2101  
2106  
2111  
2116  
2121  
2126  
2131  
2136  
2141  
2146  
2151  
2156  
2161  
2166  
2171  
2176  
2181  
2186  
2191  
2196  
2201  
2206  
2211  
2216  
2221  
2226  
2231  
2236  
2241  
2246  
2251  
2256  
2261  
2266  
2271  
2276  
2281  
2286  
2291  
2296  
2301  
2306  
2311  
2316  
2321  
2326  
2331  
2336  
2341  
2346  
2351  
2356  
2361  
2366  
2371  
2376  
2381  
2386  
2391  
2396  
2401  
2406  
2411  
2416  
2421  
2426  
2431  
2436  
2441  
2446  
2451  
2456  
2461  
2466  
2471  
2476  
2481  
2486  
2491  
2496  
2501  
2506  
2511  
2516  
2521  
2526  
2531  
2536  
2541  
2546  
2551  
2556  
2561  
2566  
2571  
2576  
2581  
2586  
2591  
2596  
2601  
2606  
2611  
2616  
2621  
2626  
2631  
2636  
2641  
2646  
2651  
2656  
2661  
2666  
2671  
2676  
2681  
2686  
2691  
2696  
2701  
2706  
2711  
2716  
2721  
2726  
2731  
2736  
2741  
2746  
2751  
2756  
2761  
2766  
2771  
2776  
2781  
2786  
2791  
2796  
2801  
2806  
2811  
2816  
2821  
2826  
2831  
2836  
2841  
2846  
2851  
2856  
2861  
2866  
2871  
2876  
2881  
2886  
2891  
2896  
2901  
2906  
2911  
2916  
2921  
2926  
2931  
2936  
2941  
2946  
2951  
2956  
2961  
2966  
2971  
2976  
2981  
2986  
2991  
2996  
3001  
3006  
3011  
3016  
3021  
3026  
3031  
3036  
3041  
3046  
3051  
3056  
3061  
3066  
3071  
3076  
3081  
3086  
3091  
3096  
3101  
3106  
3111  
3116  
3121  
3126  
3131  
3136  
3141  
3146  
3151  
3156  
3161  
3166  
3171  
3176  
3181  
3186  
3191  
3196  
3201  
3206  
3211  
3216  
3221  
3226  
3231  
3236  
3241  
3246  
3251  
3256  
3261  
3266  
3271  
3276  
3281  
3286  
3291  
3296  
3301  
3306  
3311  
3316  
3321  
3326  
3331  
3336  
3341  
3346  
3351  
3356  
3361  
3366  
3371  
3376  
3381  
3386  
3391  
3396  
3401  
3406  
3411  
3416  
3421  
3426  
3431  
3436  
3441  
3446  
3451  
3456  
3461  
3466  
3471  
3476  
3481  
3486  
3491  
3496  
3501  
3506  
3511  
3516  
3521  
3526  
3531  
3536  
3541  
3546  
3551  
3556  
3561  
3566  
3571  
3576  
3581  
3586  
3591  
3596  
3601  
3606  
3611  
3616  
3621  
3626  
3631  
3636  
3641  
3646  
3651  
3656  
3661  
3666  
3671  
3676  
3681  
3686  
3691  
3696  
3701  
3706  
3711  
3716  
3721  
3726  
3731  
3736  
3741  
3746  
3751  
3756  
3761  
3766  
3771  
3776  
3781  
3786  
3791  
3796  
3801  
3806  
3811  
3816  
3821  
3826  
3831  
3836  
3841  
3846  
3851  
3856  
3861  
3866  
3871  
3876  
3881  
3886  
3891  
3896  
3901  
3906  
3911  
3916  
3921  
3926  
3931  
3936  
3941  
3946  
3951  
3956  
3961  
3966  
3971  
3976  
3981  
3986  
3991  
3996  
4001  
4006  
4011  
4016  
4021  
4026  
4031  
4036  
4041  
4046  
4051  
4056  
4061  
4066  
4071  
4076  
4081  
4086  
4091  
4096  
4101  
4106  
4111  
4116  
4121  
4126  
4131  
4136  
4141  
4146  
4151  
4156  
4161  
4166  
4171  
4176  
4181  
4186  
4191  
4196  
4201  
4206  
4211  
4216  
4221  
4226  
4231  
4236  
4241  
4246  
4251  
4256  
4261  
4266  
4271  
4276  
4281  
4286  
4291  
4296  
4301  
4306  
4311  
4316  
4321  
4326  
4331  
4336  
4341  
4346  
4351  
4356  
4361  
4366  
4371  
4376  
4381  
4386  
4391  
4396  
4401  
4406  
4411  
4416  
4421  
4426  
4431  
4436  
4441  
4446  
4451  
4456  
4461  
4466  
4471  
4476  
4481  
4486  
4491  
4496  
4501  
4506  
4511  
4516  
4521  
4526  
4531  
4536  
4541  
4546  
4551  
4556  
4561  
4566  
4571  
4576  
4581  
4586  
4591  
4596  
4601  
4606  
4611  
4616  
4621  
4626  
4631  
4636  
4641  
4646  
4651  
4656  
4661  
4666  
4671  
4676  
4681  
4686  
4691  
4696  
4701  
4706  
4711  
4716  
4721  
4726  
4731  
4736  
4741  
4746  
4751  
4756  
4761  
4766  
4771  
4776  
4781  
4786  
4791  
4796  
4801  
4806  
4811  
4816  
4821  
4826  
4831  
4836  
4841  
4846  
4851  
4856  
4861  
4866  
4871  
4876  
4881  
4886  
4891  
4896  
4901  
4906  
4911  
4916  
4921  
4926  
4931  
4936  
4941  
4946  
4951  
4956  
4961  
4966  
4971  
4976  
4981  
4986  
4991  
4996  
5001  
5006  
5011  
5016  
5021  
5026  
5031  
5036  
5041  
5046  
5051  
5056  
5061  
5066  
5071  
5076  
5081  
5086  
5091  
5096  
5101  
5106  
5111  
5116  
5121  
5126  
5131  
5136  
5141  
5146  
5151  
5156  
5161  
5166  
5171  
5176  
5181  
5186  
5191  
5196  
5201  
5206  
5211  
5216  
5221  
5226  
5231  
5236  
5241  
5246  
5251  
5256  
5261  
5266  
5271  
5276  
5281  
5286  
5291  
5296  
5301  
5306  
5311  
5316  
5321  
5326  
5331  
5336  
5341  
5346  
5351  
5356  
5361  
5366  
5371  
5376  
5381  
5386  
5391  
5396  
5401  
5406  
5411  
5416  
5421  
5426  
5431  
5436  
5441  
5446  
5451  
5456  
5461  
5466  
5471  
5476  
5481  
5486  
5491  
5496  
5501  
5506  
5511  
5516  
5521  
5526  
5531  
5536  
5541  
5546  
5551  
5556  
5561  
5566  
5571  
5576  
5581  
5586  
5591  
5596  
5601  
5606  
5611  
5616  
5621  
5626  
5631  
5636  
5641  
5646  
5651  
5656  
5661  
5666  
5671  
5676  
5681  
5686  
5691  
5696  
5701  
5706  
5711  
5716  
5721  
5726  
5731  
5736  
5741  
5746  
5751  
5756  
5761  
5766  
5771  
5776  
5781  
5786  
5791  
5796  
5801  
5806  
5811  
5816  
5821  
5826  
5831  
5836  
5841  
5846  
5851  
5856  
5861  
5866  
5871  
5876  
5881  
5886  
5891  
5896  
5901  
5906  
5911  
5916  
5921  
5926  
5931  
5936  
5941  
5946  
5951  
5956  
5961  
5966  
5971  
5976  
5981  
5986  
5991  
5996  
6001  
6006  
6011  
6016  
6021  
6026  
6031  
6036  
6041  
6046  
6051  
6056  
6061  
6066  
6071  
6076  
6081  
6086  
6091  
6096  
6101  
6106  
6111  
6116  
6121  
6126  
6131  
6136  
6141  
6146  
6151  
6156  
6161  
6166  
6171  
6176  
6181  
6186  
6191  
6196  
6201  
6206  
6211  
6216  
6221  
6226  
6231  
6236  
6241  
6246  
6251  
6256  
6261  
6266  
6271  
6276  
6281  
6286  
6291  
6296  
6301  
6306  
6311  
6316  
6321  
6326  
6331  
6336  
6341  
6346  
6351  
6356  
6361  
6366  
6371  
6376  
6381  
6386  
6391  
6396  
6401  
6406  
6411  
6416  
6421  
6426  
6431  
6436  
6441  
6446  
6451  
6456  
6461  
6466  
6471  
6476  
6481  
6486  
6491  
6496  
6501  
6506  
6511  
6516  
6521  
6526  
6531  
6536  
6541  
6546  
6551  
6556  
6561  
6566  
6571  
6576  
6581  
6586  
6591  
6596  
6601  
6606  
6611  
6616  
6621  
6626  
6631  
6636  
6641  
6646  
6651  
6656  
6661  
6666  
6671  
6676  
6681  
6686  
6691  
6696  
6701  
6706  
6711  
6716  
6721  
6726  
6731  
6736  
6741  
6746  
6751  
6756  
6761  
6766  
6771  
6776  
6781  
6786  
6791  
6796  
6801  
6806  
6811  
6816  
6821  
6826  
6831  
6836  
6841  
6846  
6851  
6856  
6861  
6866  
6871  
6876  
6881  
6886  
6891  
6896  
6901  
6906  
6911  
6916  
6921  
6926  
6931  
6936  
6941  
6946  
6951  
6956  
6961  
6966  
6971  
6976  
6981  
6986  
6991  
6996  
7001  
7006  
7011  
7016  
7021  
7026  
7031  
7036  
7041  
7046  
7051  
7056  
7061  
7066  
7071  
7076  
7081  
7086  
7091  
7096  
7101  
7106  
7111  
7116  
7121  
7126  
7131  
7136  
7141  
7146  
7151  
7156  
7161  
7166  
7171  
7176  
7181  
7186  
7191  
7196  
7201  
7206  
7211  
7216  
7221  
7226  
7231  
7236  
7241  
7246  
7251  
7256  
7261  
7266  
7271  
7276  
7281  
7286  
7291  
7296  
7301  
7306  
7311  
7316  
7321  
7326  
7331  
7336  
7341  
7346  
7351  
7356  
7361  
7366  
7371  
7376  
7381  
7386  
7391  
7396  
7401  
7406  
7411  
7416  
7421  
7426  
7431  
7436  
7441  
7446  
7451  
7456  
7461  
7466  
7471  
7476  
7481  
7486  
7491  
7496  
7501  
7506  
7511  
7516  
7521  
7526  
7531  
7536  
7541  
7546  
7551  
7556  
7561  
7566  
7571  
7576  
7581  
7586  
7591  
7596  
7601  
7606  
7611  
7616  
7621  
7626  
7631  
7636  
7641  
7646  
7651  
7656  
7661  
7666  
7671  
7676  
7681  
7686  
7691  
7696  
7701  
7706  
7711  
7716  
7721  
7726  
7731  
7736  
7741  
7746  
7751  
7756  
7761  
7766  
7771  
7776  
7781  
7786  
7791  
7796  
7801  
7806  
7811  
7816  
7821  
7826  
7831  
7836  
7841  
7846  
7851  
7856  
7861  
7866  
7871  
7876  
7881  
7886  
7891  
7896  
7901  
7906  
7911  
7916  
7921  
7926  
7931  
7936  
7941  
7946  
7951  
7956  
7961  
7966  
7971  
7976  
7981  
7986  
7991  
7996  
8001  
8006  
8011  
8016  
8021  
8026  
8031  
8036  
8041  
8046  
8051  
8056  
8061  
8066  
8071  
8076  
8081  
8086  
8091  
8096  
8101  
8106  
8111  
8116  
8121  
8126  
8131  
8136  
8141  
8146  
8151  
8156  
8161  
8166  
8171  
8176  
8181  
8186  
8191  
8196  
8201  
8206  
8211  
8216  
8221  
8226  
8231  
8236  
8241  
8246  
8251  
8256  
8261  
8266  
8271  
8276  
8281  
8286  
8291  
8296  
8301  
8306  
8311  
8316  
8321  
8326  
8331  
8336  
8341  
8346  
8351  
8356  
8361  
8366  
8371  
8376  
8381  
8386  
8391  
8396  
8401  
8406  
8411  
8416  
8421  
8426  
8431  
8436  
8441  
8446  
8451  
8456  
8461  
8466  
8471  
8476  
8481  
8486  
8491  
8496  
8501  
8506  
8511  
8516  
8521  
8526  
8531  
8536  
8541  
8546  
8551  
8556  
8561  
8566  
8571  
8576  
8581  
8586  
8591  
8596  
8601  
8606  
8611  
8616  
8621  
8626  
8631  
8636  
8641  
8646  
8651  
8656  
8661  
8666  
8671  
8676  
8681  
8686  
8691  
8696  
8701  
8706  
8711  
8716  
8721  
8726  
8731  
8736  
8741  
8746  
8751  
8756  
8761  
8766  
8771  
8776  
8781  
8786  
8791  
8796  
8801  
8806  
8811  
8816  
8821  
8826  
8831  
8836  
8841  
8846  
8851  
8856  
8861  
8866  
8871  
8876  
8881  
8886  
8891  
8896  
8901  
8906  
8911  
8916  
8921  
8926  
8931  
8936  
8941  
8946  
8951  
8956  
8961  
8966  
8971  
8976  
8981  
8986  
8991  
8996  
9001  
9006  
9011  
9016  
9021  
9026  
9031  
9036  
9041  
9046  
9051  
9056  
9061  
9066  
9071  
9076

TABLE II-continued

| Alloy | HARDNESS AND ELECTRICAL CONDUCTIVITY COMPARISONS |        | 5 |
|-------|--------------------------------------------------|--------|---|
|       | Vickers Hardness<br>Kg/mm <sup>2</sup>           | % IACS |   |
| A126  | 178                                              | 81     |   |
| A293  | 182                                              | 79.5   |   |
| A318  | 180                                              | 80     |   |

The average values for the vanadium containing alloys are a Vickers hardness of 180 and a % IACS of 80. This compares to the 179 Vickers hardness and 83% IACS displayed by the alloy system of the present invention. It is evident from such results that the alloy system of the present invention, for equivalent hardness values, exhibits an absolute increase of 3% in IACS conductivity over alloys containing vanadium which have been utilized for the same purposes as the alloy system of the present invention. Therefore, the alloy system and processing of the present invention provides for an increase in electrical conductivity properties but not at the expense of strength or hardness properties for the alloy.

### EXAMPLE III

An alloy having a composition of 0.5% by weight chromium, 0.14% by weight zirconium, balance essentially copper was processed according to sequence (B) in Table I of Example I plus an additional 75% cold working. The strength and conductivity values for this alloy system are shown in Table III.

TABLE III

| ELECTRICAL CONDUCTIVITY AND STRENGTH COMPARISON PROPERTIES |           |               |        |  |
|------------------------------------------------------------|-----------|---------------|--------|--|
| Processing                                                 | UTS (ksi) | 0.2% YS (ksi) | % IACS |  |
| S.A. + 75% CR + 450° C/8 hrs. + 75% CR                     | 97        | 90.5          | 72.5   |  |

The results presented in Table III indicate that an alloy system similar to the alloy presented in Example I but lacking niobium does not give the desired combination of high strength and high electrical conductivity that the system of Example I with niobium exhibits in Table I. Such a system without niobium has properties which are quite similar to the literature processing results presented in Table I. Therefore, it is the combination of the novel alloy system and the processing of the present invention which provides for an increase in electrical conductivity properties but not at the expense of strength properties for the alloy.

This invention may be embodied in other forms or carried out in other ways without departing from the spirit or essential characteristics thereof. The present embodiment is therefore to be considered as in all respects illustrative and not restrictive, the scope of the invention being indicated by the appended claims, and all changes which come within the meaning and range of equivalency are intended to be embraced therein.

What is claimed is:

1. A copper base alloy which exhibits a combination of high strength and high electrical conductivity, said alloy consisting essentially of 0.05 to 1.25% by weight chromium, 0.05 to 1.0% by weight zirconium, 0.05 to 1.5% by weight niobium, balance copper.

2. A process for improving both the strength and electrical conductivity properties of copper base alloys, which comprises:

a. casting a copper base alloy consisting essentially of 0.05 to 1.25% by weight chromium, 0.05 to 1.0% by

weight zirconium, 0.05 to 1.5% by weight niobium, balance copper;

b. hot working the alloy at a starting temperature of 950°-1000° C to effect the maximum solid solution of all alloying elements;

c. rapidly cooling the alloy to maintain said maximum solid solution of all alloying elements;

d. cold working the alloy to a total reduction of at least 60%; and

e. aging said alloy at 400°-500° C for one to 24 hours.

3. A process for improving both the strength and electrical conductivity properties of copper base alloys, which comprises:

a. casting a copper base alloy consisting essentially of 0.05 to 1.25% by weight chromium, 0.05 to 1.0% by weight zirconium, 0.05 to 1.5% by weight niobium, balance copper;

b. hot working the alloy at a starting temperature of 850°-950° C;

c. solution annealing the worked alloy at a solutionizing temperature of 950°-1000° C, for a period of time sufficient to insure the maximum solid solution of all alloying elements;

d. rapidly cooling the alloy to maintain said maximum solid solution of all alloying elements;

e. cold working the alloy to a total reduction of at least 60%; and

f. aging said alloy at 400°-500° C for one to 24 hours.

4. A process as in claim 2 wherein said aging step is accomplished in cycles with said cold working, where the cycles end with either an aging or a cold working

40 step.

5. A process as in claim 2 wherein the alloy is cast at a temperature which ranges between 25° C above the melting point of the alloy up to 1300° C.

6. A process as in claim 2 wherein said rapid cooling is sufficient to cool the alloy to at least 350° C.

7. A process as in claim 3 wherein said aging step is accomplished in cycles with said cold working, where the cycles end with either an aging or a cold working step.

8. A process as in claim 2 wherein the hot working occurs at a temperature of 975°-1000° C.

9. A process as in claim 3 wherein the solutionizing temperature is 975°-1000° C.

10. A process as in claim 3 wherein the alloy is cast at a temperature which ranges between 25° C above the melting point of the alloy up to 1300° C.

11. A process as in claim 3 wherein said rapid cooling is sufficient to cool the alloy to at least 350° C.

12. A wrought copper base alloy in the worked and aged condition having high strength and high electrical conductivity properties, said wrought alloy consisting essentially of 0.05 to 1.25% by weight chromium, 0.05 to 1.0% by weight zirconium, 0.05 to 1.5% by weight niobium, balance copper.

13. An alloy as in claim 1 wherein said alloy consists essentially of 0.5 to 1.0% by weight chromium, 0.1 to 0.4% by weight zirconium, 0.1 to 0.4% by weight niobium, balance copper.

**14.** An alloy as in claim 1 wherein a small but effective amount of an element selected from the group consisting of arsenic, magnesium, cobalt, boron, calcium, cadmium and mischmetal is added to said alloy.

**15.** A process as in claim 2 wherein said alloy consists essentially of 0.5 to 1.0% by weight chromium, 0.1 to 0.4% by weight zirconium, 0.1 to 0.4% by weight niobium, balance copper.

**16.** A process as in claim 2 wherein a small but effective amount of an element selected from the group consisting of arsenic, magnesium, cobalt, boron, calcium, cadmium and mischmetal is added to said alloy of step (a).

**17.** A wrought alloy as in claim 12 wherein said alloy consists essentially of 0.5 to 1.0% by weight chromium,

0.1 to 0.4% by weight zirconium, 0.1 to 0.4% by weight niobium, balance copper.

**18.** A wrought alloy as in claim 12 wherein a small but effective amount of an element selected from the group consisting of arsenic, magnesium, cobalt, boron, calcium, cadmium and mischmetal is added to said alloy.

**19.** A process as in claim 3 wherein said alloy consists essentially of 0.5 to 1.0% by weight chromium, 0.1 to 0.4% by weight zirconium, 0.1 to 0.4% by weight niobium, balance copper.

**20.** A process as in claim 3 wherein a small but effective amount of an element selected from the group consisting of arsenic, magnesium, cobalt, boron, calcium, cadmium and mischmetal is added to said alloy of step (a).

\* \* \* \* \*

20

25

30

35

40

45

50

55

60

65

UNITED STATES PATENT AND TRADEMARK OFFICE  
Certificate

Patent No. 4,049,426

Patented September 20, 1977

W. Gary Watson and John F. Breedis

Application having been made by W. Gary Watson and John F. Breedis, the inventors named in the patent above identified, and Olin Corporation, a corporation of Virginia, the assignee, for the issuance of a certificate under the provisions of Title 35, Section 256, of the United States Code, adding the names of Brian Mravic and Stanley Shapiro as joint inventors, and a showing and proof of facts satisfying the requirements of the said section having been submitted, it is this 20th day of June 1978, certified that the names of the said Brian Mravic and Stanley Shapiro are hereby added to the said patent as joint inventors with the said W. Gary Watson and John F. Breedis.

FRED W. SHERLING,  
*Associate Solicitor.*